# EUROPEAN PATENT SPECIFICATION

(11) **EP 0 019 945 B1**
(45) Date of publication and mention of the grant of the patent: **28.08.1985**
(21) Application number: 80200322.8
(22) Date of filing: 11.04.1980
(51) Int. Cl.: C22C 11/02, H01M 4/68

(54) **Lead alloy comprising calcium and magnesium**
Kalzium- und Magnesiumhaltige Bleilegierung
Alliage de plomb contenant du calcium et du magnésium

(30) Priority: 14.05.1979 NL 7903764
(43) Date of publication of application: 10.12.1980
(73) Proprietor: SHELL INTERNATIONALE RESEARCH MAATSCHAPPIJ B.V., 2596 HR Den Haag (NL)
(72) Inventor: Baan, Diederich Jan, NL-6827 AT Arnhem (NL)
(74) Representative: Aalbers, Onno

## Description

The invention relates to lead alloy comprising calcium and magnesium. The main application of calcium-containing lead is in the form of battery lead. Further, it finds application as cable lead and as anode material in the zinc electrolysis process.

Calcium-containing lead is usually prepared by melting a lead with a purity of more than 99.9% and by subsequently adding the required alloying elements to the lead melt. This alloying step serves to impart to lead the desired mechanical properties for battery plates and grids and any other products and also to improve the castability of lead.

In the past antimony was usually added to lead. However, antimony causes self-discharge in batteries and it was therefore suggested in the prior art to replace antimony by calcium. In addition, some tin is often added to the melt. After the addition of the alloying elements, the molten lead is either made into a half-product or cast directly into the desired end-product. A half-product may consist of ingots which are remelted by the battery manufacturer and are further processed into plates and grids. The half-product may also consist of strip produced by continuous casting and/or rolling, which is further processed into plates or grids by the battery manufacturer.

Both when remelting the half-product and when remelting rejected end-products and also during the considerable period which elapses during the casting of the original melt after alloying, or of the melt obtained by remelting ingots or rejected end-products, the molten lead is in contact with the air. Now the calcium content of the melt is found to decrease gradually by oxidation of calcium, which passes as oxide into the slag layer on top of the melt. Since a certain calcium content in battery lead is desirable, the diminishing content is found to be very inconvenient. The desired calcium content is usually the maximum percentage of calcium soluble in liquid lead at the eutectic temperature (326°C). Unfortunately, it does not suffice to supply more than the desired quantity of calcium during the alloying step in order to anticipate in this manner the expected burning-off of calcium, since the degree of burning-off is difficult to predict and the presence of more calcium in the end products than can be maximally dissolved in liquid lead at the eutectic temperature (326°C) may considerably reduce the corrosion resistance of these products.

The nearest prior art comprises (i) US-A-2,306,899 which discloses lead alloys comprising 1-90 ppm of calcium and 1-90 ppm of magnesium and (ii) GB-A-499,549 which relates to lead alloys comprising 100-1000 ppm of calcium and 100-3000 ppm of magnesium, these alloys having a good composition stability after remelting and a good corrosion resistance, also when they include tin as further alloying element.

in order to solve the problems discussed hereinbefore the present invention proposes a lead alloy which comprises 1-80 ppm magnesium and 690-900 ppm calcium. It was surprisingly found that even very low percentages of magnesium in a calcium-containing lead melt almost completely inhibit the burning-off of that calcium. So far no unequivocal explanation for this phenomenon has been found. It is not or at any rate not largely so that the magnesium is sacrificed for the calcium since in order to prevent a certain quantity of calcium from being burnt off in a certain period, not a stoichiometric quantity of magnesium is required but a considerably smaller quantity of magnesium is sufficient. Neither does this smaller quantity of magnesium burn off proportionally as rapidly as the calcium would have done if no magnesium had been present in the melt.

The maximum solubility of calcium in liquid lead at the eutectic temperature (326°C) is 800 ppm. According to the invention less than 900 ppm of calcium are therefore added while moreover it is preferred to add about 700 ppm of calcium.

In the preparation of the alloy of the invention both the calcium and the magnesium can be added in elemental form, in the form of a compound or as an alloy. The percentages given in this specification are all percentages by weight and, where the relevant metal is added in the bound form, they relate to the proportion of that same metal.

In some instances difficulties may be experienced in the addition of the additives to the melt, for example because of the density of the additive (it may float on the lead melt), because of the melting point of the additive (at low melting points fewer difficulties will occur than at higher melting points) or because of the rate at which the additive dissolves in the melt.

These problems may be solved by adding the magnesium in the form of a preliminary alloy or in the form of an intermetallic compound, for example with lead (high density), or with calcium.

The invention is eminently suitable for those lead alloys which contain tin (usually less than 1%), since tin accelerates the burning-off of calcium-containing lead in a melt, so that in this instance the addition of magnesium is all the more essential.

The invention will now be illustrated by the following experiments.
1. (for comparison) A quantity of 700 ppm of calcium was added at 450°C to a quantity of 10 kg of molten lead which contained 0.39% of tin and after some time samples were taken from the melt. The results obtained are given in Table 1.
2. A quantity of 40 ppm of magnesium and 700 ppm of calcium was added at 450°C to 10 kg of molten lead which contained 0.39% of tin and some samples were taken from the melt after some time had passed. The results obtained are given in Table 1.

The calcium content was determined with an accuracy of approx. 50 ppm. It can be seen from Table 1 that the calcium content of a melt without magnesium declines rapidly and that addition of magnesium produces a change.

3. Two melts each of 10 kg of lead which contained 0.39% of tin were prepared to which the following additives were given (analysis of melt as cast):
Melt No. 3 (for comparison): 400 ppm of calcium,
Melt No. 4: 20 ppm of magnesium, 690 ppm of calcium.

The melts of lead were each remelted separately after they had been cast and analysed and the alloys thus remelted were then again cast and analysed:
Melt No. 3: 230 ppm of calcium,
Melt No. 4: 10 ppm of magnesium, 630 ppm of calcium.

This shows that the calcium content of lead decreases by remelting, but that this decrease may be greatly reduced by magnesium.
4. A number of lead/calcium/magnesium/tin alloys containing 0.35% tin were prepared and tested to determine their corrosion resistance behaviour:

These tests show that a decrease of the magnesium content favours the corrosion resistance and that an increase of the calcium content reduces the corrosion resistance. The best results are obtained with the alloys No. 3 and 5 in accordance with the present invention.

## Claims

Lead alloy comprising 1 to 80 ppm magnesium and a small amount of calcium, characterized in that the calcium content of the alloy is 690 to 900 ppm.

## Patentansprüche

Bleilegierung mit einem Gehalt an 1 bis 80 ppm Magnesium und an einer kleinen Kalziummenge, dadurch gekennzeichnet, daß der Kalziumgehalt der Legierung 690 bis 900 ppm beträgt.

## Revendications

Alliage de plomb contenant 1 à 80 ppm de magnésium et une petite quantité de calcium, caractérisé en ce que la teneur en calcium de l'alliage est de 690 à 900 ppm.
